

Dec. 27, 1949

R. S. JOHN

2,492,429

ELECTRIC TRANSLATING DEVICE

Filed Aug. 17, 1945

*Fig. 1.*



*Fig. 2.*



INVENTOR  
Robert S. JOHN  
By Clinton Wiley Schrader  
Merriam, Hoffren, Schrader

## UNITED STATES PATENT OFFICE

2,492,429

## ELECTRIC TRANSLATING DEVICE

Robert S. John, Waukegan, Ill., assignor to Pfanz-  
stiehl Chemical Company, a corporation of  
Illinois

Application August 17, 1945, Serial No. 610,975

14 Claims. (Cl. 201—75)

1

This invention relates to a translating device and particularly to a method of making a translating device for translating mechanical variations into electrical variations, and the product prepared thereby.

One object of this invention is to provide an improved translating device made of a flexible material and having a coating forming an electrical path with the resistance being varied by strain. Another object is to provide an improved method of making such a translating device so that the resulting product will give uniform results over a wide range of frequencies. Still another object is to provide a simple, efficient, and rapid method of producing such a translating device so that any desired characteristics may be given thereto. Other objects will be apparent from the detail description given hereinafter.

The particular translating device described herein is a phonograph pick-up of the same general nature as those shown in the Kenneth J. Germeshausen Patents No. 2,329,526, 2,373,676, and 2,380,514, but it will be understood that the processes here disclosed are applicable to translating devices in any field where a mechanical movement is to be translated into an electrical variation.

In practicing this invention I provide a flexible base member having at least one surface of a flexible insulating material with this base member being intended to be subjected to mechanical variation. A coating of finely divided particulate material suspended in a solvent for the flexible insulating surface is applied to this surface. The particulate material used is one that is capable of forming a layer whose electrical resistance is varied by strain. This coating is dried, and then a final coating of flexible insulating material is applied over the strain-sensitive coating.

The base member may be made of a flexible insulating material throughout, and this is preferably a synthetic elastomer having a low modulus of elasticity, such as polystyrene, polymerized methyl methacrylate, or the like. The strain-sensitive material is preferably very finely divided graphite, such as that made in an electric furnace, and this graphite is applied by suspending it in a solvent for the synthetic elastomer. Where the elastomer is polystyrene carbon tetrachloride is an excellent solvent, as it softens the polystyrene so that the graphite will be held thereon, but evaporates so rapidly that there is no undue penetration and substantially no swelling action on the polystyrene. Other solvents for polystyrene include toluene, ethyl benzene, ethyl

2

acetate, turpentine, dioxane, gasoline, ethylene chloride, Cellosolve acetate, and paradichlorobenzene. For any given synthetic elastomer a solvent should be chosen that softens the elastomer sufficiently to form an adhesive surface upon which the graphite may be deposited, but should also have a low boiling point so that the solvent will readily evaporate before penetrating very deeply into the elastomer.

10 In making the strain-sensitive coating of graphite on polystyrene, a suspension of graphite in 2 to 3 times its volume of carbon tetrachloride is prepared. The polystyrene surface is then dipped in this suspension and allowed to dry quietly at preferably not more than 70° F. for at least an hour, and preferably for as much as 24 hours, in an atmosphere having low humidity, not over 30% and preferably between 10% and 20%. The extra drop that clings to the dipped coating should not be wiped off, but should be evenly distributed, such as by holding the polystyrene with the coating in a horizontal position, and slowly rotating it under conditions where it is substantially entirely free from vibration, as 15 on spring-mounted drying apparatus. One dipping will produce a very opaque coating of rather high resistance. If the resistance is to be brought down to a lower predetermined value successive 20 dipping are made in the same solution, with each coating dried thoroughly before the next is applied. My preferred method provides a coating 25 on spring-mounted drying apparatus. One dipping will produce a very opaque coating of rather high resistance. If the resistance is to be brought down to a lower predetermined value successive dipping are made in the same solution, with each coating dried thoroughly before the next is applied. My preferred method provides a coating having desired resistance characteristics with freedom from noise in operation.

30 After the strain-sensitive coating has been made, the desired circuit is scribed out and the plastic with the graphite coating is then dipped in a fairly thin lacquer solution and dried. This gives an overall covering of flexible insulating material. One lacquer that has been used is made by the Zapon Brevolite Corporation, and 35 is known as XL-44 Lacquer. The active ingredient is elemi, a natural resin. The lacquer to be used should be one that is flexible and that will not cause distortion of the plastic base member. Lacquers other than that mentioned have 40 these properties and may be used.

45 When the polystyrene or other synthetic elastomer is successively dipped in the graphite suspension, each dipping should be made as rapidly as possible, so that some of the graphite put on in previous dippings is not washed off. The drying which follows each dipping should be done in a dust-free and dry atmosphere, free from drafts, and should be done at a temperature 50 not substantially greater than 70° F. The final

drying should be continued for at least 24 to 48 hours, as in this time the resistance drops to a final value and becomes quieter.

The translating device which is the subject of this invention has the flexible portion containing the graphite layer or other strain-sensitive material, and usually has another rigid portion that is not flexed. This rigid portion ordinarily carries binding posts or the like to which electrical leads may be fastened so as to complete the electrical circuit through the strain-sensitive coating. In the prior patents mentioned hereinabove this rigid portion was coated with a graphite layer to complete the circuit. The graphite layer, however, resisted flow of electricity where such resistance was not needed. It has been discovered, however, that a superior translating device will be produced if the rigid portion of the device is coated with a layer of freely-conducting material which contacts the layer of strain-sensitive material in order to complete the electrical circuit. The conducting material preferably is an oxide-free suspension of metal in a solvent for the synthetic elastomer.

One of the best metals for making conductive coatings is commercially precipitated silver free of silver oxide and having substantially no particles larger than 200 mesh. This silver may be suspended in 2 or 3 times its volume of solvent and applied to the base member with a brush in the desired path. When the elastomer is polystyrene the solvent may be carbon tetrachloride. The coating of powdered metal should be thick enough to be opaque, usually not less than 0.001 inch.

One embodiment of this invention is shown in the accompanying drawings. Of the drawings Fig. 1 is a side elevation of a translating device made according to the method of this invention; and Fig. 2 is a plan view of this translating device.

The translating device 10 shown in the accompanying drawings comprises a rigid portion 11 adapted to be mounted on a tone arm of a phonograph or the like, and a beam 12 extending therefrom. At the end of the beam there is located a rigidly mounted needle or stylus 13 adapted to engage the grooves of a record. The beam 12 has a coating of graphite 14 arranged in the form of a path extending from near the base 11 out toward the end of the beam 12 and back to the base. The beam 11 has two holes 15 and 16 by which the device may be mounted and which may also be used to provide electrical connections to the resistance path. From each of these holes there is provided a layer of silver 17 with each layer connecting to one end of the graphite path. Thus a complete circuit is formed extending toward the end of the beam 12 that holds the needle 13.

In making the graphite layer 14 the beam 12 is immersed in a graphite suspension of electrically produced graphite in 2 or 3 times its volume of carbon tetrachloride. The beam is immersed in the suspension a plurality of times, with each immersion followed by complete drying for at least one hour, at a temperature not greater than 70° F. These successive immersions are continued until the overall resistance of the graphite layer is five to eight thousand ohms before scribing and 30,000 to 35,000 ohms after the circuit paths have been scribed thereon. This circuit path may be on one or more sides of the beam. The silver layer on the rigid portion 11 of the translating device is prepared by brushing

on a suspension of finely divided oxide-free silver in carbon tetrachloride. The silver is brushed on in the desired path and a sufficient quantity is applied so that the silver layer will be at least 0.001 in. thick. The rigid portion is then dried for at least one hour at not more than 70° F.

After the silver and graphite layers have been applied these layers are covered with a solution of lacquer as described above. The lacquer layer 10 is then dried at a temperature not greater than 70° F. The graphite layer which prior to the lacquer coating had a resistance of 30,000 to 35,000 ohms, should now have a resistance of 60,000 to 80,000 ohms.

The silver coatings may be lightly burnished before the lacquer is applied, as this improves the conductivity of the silver layers.

The solvent used in making the various suspensions employed in practicing this invention should be one which dissolves the flexible material readily but has a rapid rate of evaporation so that the penetration of the solvent will be very slight. One of the best solvents for use with polystyrene base members is carbon tetrachloride, while acetone is an excellent solvent when polymerized methyl methacrylate is used to make the base member. The lacquer used should be one that is freely flexible at all ordinary temperatures, and that has no distorting effect on the base member.

These lacquers, as well as the solvents for the various flexible materials that may be used in making the translating devices, and their uses are well understood by those skilled in the art.

35 While I have shown and described certain embodiments of my invention, it is to be understood that it is capable of many modifications. Changes, therefore, in the construction and arrangement may be made without departing from 40 the spirit and scope of the invention as disclosed in the appended claims.

I claim:

1. The method of making a translating device for translating mechanical variations into electrical variations which comprises providing a flexible base member having at least one surface of a flexible insulating material, said base member being one that is to be subjected to mechanical variation, applying to said surface a coating of a finely divided particulate material suspended in a solvent which acts as a solvent for the flexible insulating surface with said particulate material being capable of forming a layer whose electrical resistance is varied by strain, drying the coating at a temperature not substantially above 70° F., and applying over the coating a layer of flexible insulating material.

2. The method of claim 1 wherein the suspension is maintained at a temperature not substantially above 70° F.

3. The method of claim 1 wherein the flexible insulating surface is a synthetic elastomer and the solvent is one that has a substantially non-swelling action on the flexible insulating material and that has a rapid rate of evaporation.

4. The method of making a translating device for translating mechanical variations into electrical variations which comprises providing a flexible base member having at least one surface of a synthetic elastomer, said base member being one that is to be subjected to mechanical variation, applying to said surface a coating of finely divided graphite suspended in a solvent which acts as a solvent for the elastomer while maintaining the suspension at a temperature not sub-

stantially above 70° F., said solvent being one that has a substantially non-swelling action on the elastomer and that has a rapid rate of evaporation, drying the coating at a temperature not substantially above 70° F. and at low humidity, applying over the coating a solution of a flexible insulating material, and drying.

5. The method of claim 4 wherein the synthetic elastomer is polystyrene and the solvent is carbon tetrachloride.

6. The method of claim 4 wherein the solution of flexible insulating material is a lacquer that has substantially no effect on the dimensions of the synthetic elastomer.

7. The method of making a translating device for translating mechanical variations into electrical variations which comprises providing a base member of polystyrene that is to be subjected to mechanical variation, applying to at least one surface of said base member a coating of finely divided graphite suspended in carbon tetrachloride that is maintained at a temperature not substantially above 70° F., drying at a temperature not substantially above 70° F. and at low humidity, applying over the coating a lacquer that has substantially no effect on the dimensions of the polystyrene, and drying.

8. The method of claim 7 wherein the graphite is applied to the base member by a plurality of dipping operations with substantially complete drying of each coating before applying the next one, with the dipping operations being continued until there is a final resistance of 30,000 to 35,000 ohms, after scraping and scribing.

9. The method of making a translating device for translating mechanical variations into electrical variations which comprises providing a flexible base member having at least one surface of a flexible insulating material, said base member being one that is to be subjected to mechanical variation, applying to said surface a coating of a finely divided particulate material suspended in a solvent which is a solvent for the flexible insulating surface by successive applications of said suspension with each application followed by drying, said particulate material being capable of forming a layer whose electrical resistance is varied by strain, and applying over the final coating a layer of flexible insulating material.

10. The method of claim 9 wherein each application is an immersion and is dried at a temperature not substantially above 70° F. for approximately 24 hours.

5 11. The method of claim 9 wherein the suspension is maintained at a temperature not substantially above 70° F., and each immersion is dried at a temperature not substantially above 70° F. for approximately 24 hours.

10 12. The method of making a translating device for translating mechanical variations into electrical variations which comprises providing a base member of polystyrene having one portion to be subjected to flexing and another portion to be held substantially rigid, coating the flexible portion with graphite suspended in carbon tetrachloride, drying, coating the rigid portion with a suspension of finely divided oxide-free silver in carbon tetrachloride with no particles of the silver being larger than 200 mesh, drying, said coatings overlapping at their adjacent edges to form a continuous electrical path, covering said coatings with a lacquer, and drying.

15 13. The method of claim 12 wherein the suspensions are maintained at a temperature not substantially above 70° F., and the coatings are dried at a temperature not substantially above 70° F.

20 14. The method of claim 4 wherein the solution of flexible insulating material causes the resistance of the coating of graphite to be substantially doubled.

ROBERT S. JOHN.

#### 35 REFERENCES CITED

The following references are of record in the file of this patent:

#### UNITED STATES PATENTS

| 40 | Number    | Name          | Date          |
|----|-----------|---------------|---------------|
|    | 1,985,166 | Haroldson     | Dec. 18, 1934 |
|    | 2,252,464 | Kearns et al. | Aug. 12, 1941 |
|    | 2,373,676 | Germeshauser  | Apr. 17, 1945 |
|    | 2,440,691 | Jira          | May 4, 1948   |

45

#### FOREIGN PATENTS

| Number  | Country       | Date          |
|---------|---------------|---------------|
| 211,324 | Great Britain | Feb. 21, 1924 |